

March 5, 1957

H. J. HAMJIAN ET AL

2,783,504

METHOD OF FORMING ARTICLES FROM COMMINUTED MATERIAL

Filed May 6, 1953

2 Sheets-Sheet 1



Fig. 5

*INVENTORS*  
*Harry J. Hamjian*  
*Falih N. Darmara*

BY

Hyde, Meyer, Baldwin & Doran  
ATTORNEYS

March 5, 1957

H. J. HAMJIAN ET AL

2,783,504

METHOD OF FORMING ARTICLES FROM COMMINUTED MATERIAL

Filed May 6, 1953

2 Sheets-Sheet 2



Fig. 6



Fig. 7



Fig. 8



Fig. 9



Fig. 10

INVENTORS

Harry J. Hamjian  
Falah N. Darmara

BY

Hyde, Meyer, Baldwin & Doran  
ATTORNEYS

1  
2,783,504**METHOD OF FORMING ARTICLES FROM  
COMMUNINATED MATERIAL**

Harry J. Hamjian, Whitesboro, and Falih N. Darmara,  
New Hartford, N. Y., assignors to Utica Drop Forge  
& Tool Corporation, Utica, N. Y., a corporation of  
New York

Application May 6, 1953, Serial No. 353,386

2 Claims. (Cl. 18—59.5)

This invention relates to novel and improved methods and means for manufacturing articles directly from comminuted materials. It particularly relates to improvements in the art of forming shaped articles of intricate contour directly from comminuted materials without the intervention of intermediate forming steps such as machining, grinding, or the like.

While not specifically limited thereto, our novel and improved process will be described as applied to the formation of articles from high temperature heat resistant metal powders, such as the silicon carbides, or metalloid powders or mixtures thereof with other suitable refractory metal or metalloid powders. It should be borne in mind, accordingly that when we describe the formation of articles from such powders we do not intend to be limited thereto, the scope of the invention being defined by the claims hereinafter appended.

As is known to those skilled in this art, the formation of articles from compressed powders of the refractory metals and carbides has followed two general methods of approach. In one such method the powders were compressed by a ram operating in conjunction with a die enclosure, and the powders were thus compressed into cylindrical, polyhedral, or similar blocks. These blocks were then sintered at high temperature. The ultimate desired shapes were then "carved" out of such blocks by grinding or machining steps.

In a second method a die was provided wherein the inner wall of the cavity was shaped to generally conform to the outer wall of the ultimate article, as in a mold for molten metal, and the powdered or comminuted particles were then pressed into the die cavity by a ram capable of exerting tremendous pressure. Obviously for a shape of even average complexity the die must be a multi-part one, so as to be separable to permit removal of the article, and undercut contours are extremely difficult to make in this way without multiplying inordinately the number of die parts. Again, in this method, the pressed article is sintered.

As is also well known in this art there is a shrinkage factor on sintering which results in a linear shrinkage of the article to an extent varying with a number of factors, including the particular axis on which the shrinkage is measured with relation to the direction of ram pressure, the particle size, the temperature of sintering, etc., and this shrinkage in the case of carbides may amount to between fifteen and eighteen percent, linearly, or forty to fifty percent, volumetrically. This must be compensated for in calculating the die dimensions.

Even when an article was made to the desired shape in a metal die under ram pressure applied either directly on an exposed surface of the powder or on a movable die part, a substantial amount of finish grinding or machining was always required in the prior art practices.

One of the disadvantages of article production as above described was the tremendous cost of the final shaping operations, whether done by one or the other of the methods described. The cemented carbides are extremely hard

after sintering, and must be machined or ground by special tools or grinding wheels which are themselves at least as hard as the object on which they operate. The portion of the work piece which is ground or cut away constitutes an expensive loss, and the tools do not have a long working life.

In an obvious admission that these methods were economically unsound, one manufacturer has attempted to solve the problem, at least in part, by first compressing the powders, then giving the compressed block or shaped article an initial partial sintering, then shaping the partially sintered material to approximately the final contour, then finishing the sintering, and finally completing the machining operation. Since a final machining step is not avoided, at least where accuracy of tolerances is needed, the solution is not completely satisfactory although some stock can be removed while in a relatively soft condition.

Further, as is known to those skilled in this art, the use of mechanical pressure, as heretofore characterized, produces uneven surface hardness, and uneven penetration of the hardening force along differently oriented axes with respect to the direction of ram pressure application and the shape of the article. This is especially true where articles are being formed in contoured metal dies wherein certain surface zones of the article are "sheltered" from the maximum pressure by die projections, etc.

Some attempts have been made in avoidance of this last-named difficulty by putting the refractory powders in a flexible bag and subjecting the bag to hydrostatic pressure, but here again the final lump of material required expensive machining or grinding operations, and as the material is cut away there arises considerable variation in surface hardness.

The main reason why this particular art has maintained a commercial position despite the above-named and other difficulties is that there exist situations in which the physical properties of an article formed from cemented carbides or refractory metals are so necessary in some specific application that the customer will pay practically any asking price for the finished article.

An object of the present invention is to provide a method of forming articles directly from metal powders with such dimensional accuracy that they conform to normal dimensional tolerances, and final finishing steps, if ever required, are of such minor character that they do not materially add to the cost of the article. Usually, the accuracy of dimension of articles made by our process is in the order of hundredths of an inch, with excellent accuracy of detail. Occasionally, if accuracy in thousandths is required, a minor amount of finish grinding suffices.

A further object of the invention is to provide a method of producing articles as defined in the last preceding paragraph wherein the density throughout the finished article is uniform to a high degree.

A further object of the invention is to produce articles as defined in the last two preceding paragraphs by means of hydrostatic pressure effective peripherally on a flexible die or mold, the interior contour of which is shaped to conform to the exterior contour of the ultimate article.

A further object of the invention is to produce shaped articles with undercuts and intricate contours, directly from comminuted powders in such way that the compressed article can be readily removed from the die.

A further object of the invention is to produce shaped articles directly from metal powders by hydrostatic pressure in molds of such character that die cost and die wear are reduced to a minimum.

Further objects and advantages will be apparent from a study of the following description of the invention, in conjunction with the accompanying drawings, in which

Fig. 1 is a diagrammatic sketch, in simplified form, showing structural elements such as were used in the compression of metal powders in the prior art.

Fig. 2 is a pictorial representation of density variation in the cross section of a polyhedral block made by means of the apparatus shown in Fig. 1.

Fig. 3 is a diagrammatic showing of a specimen under hydraulic pressure in accordance with the principle outlined in the description hereinbelow.

Fig. 4 is a diagrammatic sectional showing of a hollow flexible mold having a powder charge therein, and closure means thereon.

Fig. 5 is a diagrammatic showing of a metal die, a cavity for hydraulic fluid, a powder-containing mold in the cavity, and means for applying hydrostatic pressure within the cavity.

Fig. 6 is a perspective view of a four-bladed helical cutter of a type susceptible of ready manufacture by our invention.

Fig. 7 is a fragmentary perspective view of a flexible mold and closure suitable for use in making the cutter shown in Fig. 6.

Fig. 8 is a perspective view of a chuck wrench susceptible of ready manufacture by our invention.

Fig. 9 is a fragmentary perspective view of a flexible mold and closure suitable for use in making the wrench shown in Fig. 8.

Fig. 10 is a showing similar to Fig. 5, but in which a resilient insert has been substituted for a hydraulic fluid.

Referring now to the drawings, in generally numerical order as this description proceeds, we show a metal die 10 which has a bored aperture 11 therein, adapted to slidably receive a lower plunger or ram 12 and an upper plunger or ram 13. As exemplary of one preferred process of the prior art, comminuted metal powder 14 is poured into the aperture, on top of plunger 12, and one or both plungers are advanced towards each other within die 10 so as to compress the material. Such material is thus compressed to a volume exemplified by the space between the broken lines A, after which the plungers are appropriately moved to eject the resulting block of compressed material. The said block is then sintered for an appropriate time, in a protective atmosphere at a suitable temperature (dependent of course on the alloy or metal powder composition) to promote a firm inter-molecular bond between the particles.

Fig. 2 pictorially represents one such block 15 which has been sintered, cut vertically, and suitably etched to indicate the effect of the ram pressure on the internal structure, the pressure having been applied in the direction of the arrows "P." The zones 15a and 15b are of roughly plano-convex shape, which may here be termed for convenience "lenticular," and plainly indicate that the pressure at the center was effective to a maximum extent, the effect falling off gradually towards the peripheral face 15c of the block. The central zone 15d, of double-concave contour, represents an area of reduced density.

From a consideration of Figs. 1 and 2 it will be evident that in the prior art process just described the powdered material around the inner die periphery, by reason of friction on the die wall, and because there is only a limited number of directions to go, namely in a 90° quadrant downwardly and towards the center, will tend inevitably to take on the lenticular density characteristics just described. Obviously when an article of irregular shape is "carved" from the block 15, the cuts or ground out hollows extending to varying depths, there will result an article of varying surface hardness depending on the depth of penetration and the location of penetration. This is quite undesirable where a uniform hardness is required by the particular application.

Fig. 3 represents, pictorially, a very desirable type

of pressure application such as has been used in the prior art to achieve an even surface density in a lump of material. The cube 16 in this case represents a pliable closure such as a bag filled with comminuted metal powder and dropped into a strongly built die or closure 17 filled with liquid 18 such as oil or the like. Pressure is then applied to the liquid by means of the piston 19 and, the pressure being hydraulic, is effective equally in all directions as indicated by the arrows. As previously explained, even this method is expensive, since the final article must be machined or ground out of the block thus produced.

The economies which we have as one of our objects result from the achievement of a fully compressed structure in an article formed to final shape during the initial pressing operation, the density being uniform throughout at points equidistant from the article surface.

Since it is apparent that one of the most fundamental problems of this art is that of compacting the powder to final shape, with uniform internal structural density, and since it has been impossible in the past to achieve the final shape of the article without extremely expensive final shaping operations on the more refractory and harder metals and alloys, it occurred to us that what was needed was to develop an inexpensive but accurately contoured mold upon which hydrostatic pressure could be used in such way that the pressure is as fully effective on the comminuted metals as if the mold did not intervene.

After extensive study and experimentation we have developed a process which greatly extends the field of powdered metal compression into accurately formed yet inexpensively produced articles.

Our process comprises the use of a soft elastic mold made from rubber or rubber-like material. Such mold may be formed around a pattern identical in shape with the article to be formed except of course that compression shrinkage and eventual sintering shrinking must be allowed for, and the pattern and mold made sufficiently oversize to compensate for such shrinkages. In one method of making the mold liquid rubber was cast around the pattern, and stripped off after solidification. Obviously an aperture must exist to permit removal of the pattern and insertion of the powdered material, and the mold wall must be sufficiently strong to retain its contour when filled with comminuted materials. This method of manufacturing the mold permits the existence of undercuts and other surface irregularities which would be economically impractical to form in a rigid mold, and thereafter it would be impossible to remove the compressed article from a rigid mold.

The pattern may be made from a number of rigid materials such as wood, ferrous metal, the low melting point metals such as lead, bismuth, antimony, tin, etc., and alloys thereof, or even wax. In case of the low melting point alloys or wax, the pattern can be removed from the mold by melting, which permits even more intricately-shaped contours with involved undercuts to be used for the manufacture of the pliable mold.

Fig. 4 shows, in vertical section, a rubber mold 20 having a comminuted metal charge 21 therein. It is shown as provided with offsets or ears 21a and 21b which would render it impossible to remove the final article from a rigid die, but an inexpensive rubber mold can be stripped or cut therefrom. This showing of Fig. 4 is merely diagrammatic, and the rubber wall is made thick enough to hold its shape in actual practice, and flexible enough to allow sufficient compression of the powder to the pressed shape of the final article.

When the mold of Fig. 4 is filled with powder, it may be placed in a vacuum chamber and air evacuated therefrom since air in the interstices of the powder forms voids or porosity in the final article. A closure 22 is then sealed thereon, or otherwise attached so as to seal against

hydrostatic pressure. The sealed mold is dropped into a dead end bore 23 of a die 23a (Fig. 5) in which there is a hydraulic fluid. Above the fluid is a piston 24 propellable by a plunger 25. Between the plunger and piston is a sealing washer 26. The manner of use is obvious from what has just been described. When heavy pressure is applied to the hydraulic fluid it produces hydrostatic pressure on the yieldable mold and consequently on the powdered material in the mold. The effect of such pressure has been discussed hereinabove. Again, as in previous drawings, the showing in Fig. 5 has omitted many mechanical details necessary in practice, but not at all necessary for an understanding of the present invention.

Fig. 6 shows a rotary cutter 28 with helical teeth 29, obviously difficult or impossible to produce by using a rigid die, but well adapted for forming in a flexible-shaped die such as shown in Fig. 7. Fig. 8 shows a chuck wrench having a plain cylindrical shank 31 and a bevel-gear nosepiece 32. This is easily reproducible from the mold 33 in Fig. 9. The mold cavities of Figs. 7 and 9 are shown a noticeable amount oversize with respect to the articles respectively formed therein, merely as an indication that a predetermined relationship exists, having in mind the known compression shrinkage and sintering shrinkage of the particular material. In the sintering process, of course, a true inter-molecular bond develops between the closely packed metallic particles.

A remarkable and useful feature of our process as above described is that the article which emerges from the sintering step is an exact replica of the pattern, except for the linear and volumetric shrinkage.

Fig. 10 shows an embodiment wherein a conventional steel die 35 has a shaped insert 36 therein of rubber or rubber-like material. There can then be a lower anvil or plunger 37 and an upper plunger 38. Compression of the powder 39 produces a quasi-hydrostatic pressure in the material compacted into the mold aperture. Die wear costs can be reduced by this method since the insert 36 is replaceable at any time.

The method above described is the most economical method so far developed for reproducing small parts, of accurate contour and even density and in large numbers. Non-miscible metals may be alloyed, the porosity may be controlled, the chemical analysis may be very accurately fixed, and laminated combinations and metal-ceramic mixes may be achieved. As suitable materials we may mention molybdenum, tungsten, the carbides of said metals, titanium, zirconium, etc. These can be satisfactorily sintered at about two-thirds of their respective melting points, and eutectic temperatures should be borne in mind in mixing and sintering mixtures of metals.

In the manufacture of intricate parts in large numbers, savings of about ninety percent may be effected under the cost of the older method of using rigid dies and mechanical rams which must be followed by tedious shaping steps.

Not much has been said so far of the manufacture of articles from the non ferrous metals, for example aluminum and its alloys. In prior art methods aluminum was not usually used as a material for powder compression, since the pressing problem caused by material sticking to the dies makes powder metallurgical methods more expensive than conventional casting or mechanical deformation methods. Recent developments have shown that the oxide layer on aluminum particles, if properly

controlled, allows the fabrication of a new aluminum alloy from such powder which has exceptional high-temperature mechanical properties above the softening point of the normal aluminum alloys.

With this most recent development, attention has been given to the development of new techniques for pressing this material in order to eliminate the die sticking problem. Our solution lies in the hydrostatic pressure of pre-forms and articles in pliable molds.

The equipment problem is simplified since one hydrostatic die of adequate capacity, equivalent to the die 23a of Fig. 5, can accommodate simultaneously a number of molds for articles of varied sizes and shapes.

As in previous practices in compressing of articles from comminuted metals there is a practical upper limit to the size of articles which can be produced, of adequate overall density and uniform hardness at points equidistant from the outer surface.

In the present application the term "refractory material" is intended to include carbides such as silicon and tungsten carbide, as well as the high melting point metals such as molybdenum, tungsten, titanium and vanadium and their alloys and compounds and mixtures thereof.

What we claim is:

- 25 1. A process of forming an article having surface irregularities such as undercuts and the like, comprising providing a hollow mold formed from resilient material, said mold having walls of a thickness adequate to be self-supporting, forming the wall of the casting cavity of said mold to be complementary in contour to that of the article surface with respect to said irregularities and undercuts, but sufficiently oversize to compensate for article shrinkage during formation thereof, filling said mold with comminuted refractory material, placing said mold in a closure with sufficient liquid to immerse said mold completely, applying hydrostatic pressure to said liquid until said comminuted material is compressed to solidity and to the size of the final article, and stripping said mold from said article while maintaining said mold intact.
- 30 2. A process of forming an article having surface irregularities such as undercuts and the like, comprising providing a hollow mold formed from resilient material, said mold having walls of a thickness adequate to be self-supporting, forming the wall of the casting cavity of said mold to be complementary in contour to that of the article surface with respect to said irregularities and undercuts, but sufficiently oversize to compensate for article shrinkage during formation thereof, filling said mold with comminuted refractory material, placing said mold in a closure with sufficient liquid to immerse said mold completely, applying hydrostatic pressure to said liquid until said comminuted material is compressed to solidity and to the size of the final article, and stripping said mold from said article while maintaining said mold intact.
- 35 3. A process of forming an article having surface irregularities such as undercuts and the like, comprising providing a hollow mold formed from resilient material, said mold having walls of a thickness adequate to be self-supporting, forming the wall of the casting cavity of said mold to be complementary in contour to that of the article surface with respect to said irregularities and undercuts, but sufficiently oversize to compensate for article shrinkage during formation thereof, filling said mold with comminuted refractory material, placing said mold in a closure with sufficient liquid to immerse said mold completely, applying hydrostatic pressure to said liquid until said comminuted material is compressed to solidity and to the size of the final article, and stripping said mold from said article while maintaining said mold intact.
- 40 4. A process of forming an article having surface irregularities such as undercuts and the like, comprising providing a hollow mold formed from resilient material, said mold having walls of a thickness adequate to be self-supporting, forming the wall of the casting cavity of said mold to be complementary in contour to that of the article surface with respect to said irregularities and undercuts, but sufficiently oversize to compensate for article shrinkage during formation thereof, filling said mold with comminuted refractory material, placing said mold in a closure with sufficient liquid to immerse said mold completely, applying hydrostatic pressure to said liquid until said comminuted material is compressed to solidity and to the size of the final article, and stripping said mold from said article while maintaining said mold intact.
- 45 5. A process of forming an article having surface irregularities such as undercuts and the like, comprising providing a hollow mold formed from resilient material, said mold having walls of a thickness adequate to be self-supporting, forming the wall of the casting cavity of said mold to be complementary in contour to that of the article surface with respect to said irregularities and undercuts, but sufficiently oversize to compensate for article shrinkage during formation thereof, filling said mold with comminuted refractory material, placing said mold in a closure with sufficient liquid to immerse said mold completely, applying hydrostatic pressure to said liquid until said comminuted material is compressed to solidity and to the size of the final article, and stripping said mold from said article while maintaining said mold intact.
- 50 6. A process of forming an article having surface irregularities such as undercuts and the like, comprising providing a hollow mold formed from resilient material, said mold having walls of a thickness adequate to be self-supporting, forming the wall of the casting cavity of said mold to be complementary in contour to that of the article surface with respect to said irregularities and undercuts, but sufficiently oversize to compensate for article shrinkage during formation thereof, filling said mold with comminuted refractory material, placing said mold in a closure with sufficient liquid to immerse said mold completely, applying hydrostatic pressure to said liquid until said comminuted material is compressed to solidity and to the size of the final article, and stripping said mold from said article while maintaining said mold intact.
- 55 7. A process of forming an article having surface irregularities such as undercuts and the like, comprising providing a hollow mold formed from resilient material, said mold having walls of a thickness adequate to be self-supporting, forming the wall of the casting cavity of said mold to be complementary in contour to that of the article surface with respect to said irregularities and undercuts, but sufficiently oversize to compensate for article shrinkage during formation thereof, filling said mold with comminuted refractory material, placing said mold in a closure with sufficient liquid to immerse said mold completely, applying hydrostatic pressure to said liquid until said comminuted material is compressed to solidity and to the size of the final article, and stripping said mold from said article while maintaining said mold intact.

#### References Cited in the file of this patent

#### UNITED STATES PATENTS

|    |           |             |               |
|----|-----------|-------------|---------------|
| 60 | 1,081,618 | Madden      | Dec. 16, 1913 |
|    | 1,226,470 | Coolidge    | May 15, 1917  |
|    | 1,981,719 | Comstock    | Nov. 20, 1934 |
|    | 1,983,602 | Daubenmeyer | Dec. 11, 1934 |
|    | 2,220,018 | McKenna     | Oct. 29, 1940 |
| 65 | 2,298,908 | Wentworth   | Oct. 13, 1942 |